

**3,241,966**  
**BLEACH FIXING OF PHOTOGRAPHIC**  
**SILVER IMAGES**

Max Heilmann, Cologne-Flittard, Hanswilli von Brachel, Cologne-Sulz, and Hans Holtschmidt, Cologne-Stammheim, Germany, assignors to Agfa Aktiengesellschaft, Leverkusen, Germany, a corporation of Germany  
 No Drawing. Filed June 9, 1961, Ser. No. 140,170  
 Claims priority, application Germany, June 14, 1960,

A 34,882

3 Claims. (Cl. 96—60)

This invention relates to a process for bleach fixing of photographic silver images as well as to a bleach fixing bath.

According to German Patent Specification No. 866,605 the bleach fixing of photographic silver images is achieved by means of a bleach fix bath containing in addition to the known fixing agents for silver halide, a complex salt of trivalent iron with an organic acid of the following general formulae:



in which X represents



and

$\text{R}_1$ ,  $\text{R}_2$ , and  $\text{R}_3$  represent hydrocarbon radicals which may be substituted and  $\text{R}_3$  may also represent hydrogen, and in which  $\text{R}_4$ ,  $\text{R}_5$  and  $\text{R}_6$  represent bivalent hydrocarbon radicals which may again be substituted. Examples of suitable organic acids are ethylenediamine tetra-acetic acid, nitrilotriacetic acid, malonic acid, ethyl malonic acid, tartaric acid, malic acid, fumaric acid, diglycolic acid, ethylenimino-dipropionic acid, ethylene dithioglycolic acid and dithioglycolic acid. These bleach fix baths are highly stable and are used, in particular, for the production of multicoloured images by the colour development process. Nevertheless, these baths have the disadvantage that they do not always completely bleach out the silver images at the areas of highest density.

It is known from German patent specification No. 966,410 that it is possible to improve the effectiveness of the aforementioned bleach fix baths without affecting their stability by adding a polyethylene oxide and/or a derivative thereof to them. For this purpose, water-soluble polyethylene oxides are used, for example, polyethylene oxides of the general formulae:



In these formulae,  $\text{R}_1$  represents a hydrogen atom or a substituted or unsubstituted alkyl, aryl, aralkyl, acyl, aroyl or heterocyclic radical;  $\text{R}_2$  and  $\text{R}_3$ , which may be the same or different, each represent a hydrogen atom, a substituted or unsubstituted alkyl, aryl, aralkyl, acyl, aroyl or heterocyclic radical or the group— $(\text{CH}_2\text{CH}_2\text{O})_n\text{R}_4$ , wherein  $\text{R}_4$  is a hydrogen atom or a substituent suitable for the etherification or esterification of an —OH group and  $x$ ,  $y$ ,  $z$  and  $n$  are integers. Examples of water-soluble polyethylene oxides which increase the bleaching capacity of bleach fix baths are polyethylene oxides consisting of

from 10 to 120 mols of ethylene oxide; reaction products of fatty alcohols, for example oleyl alcohol, with from 60 to 100 mols of ethylene oxide; reaction products of lauric acid with from 10 to 20 mols of ethylene oxide; reaction products of trimethylol propane with ethylene oxide, which have an average molecular weight of 4000; reaction products of ammonia with from 20 to 30 mols of ethylene oxide; and reaction products of dimethylamine with from 50 to 70 mols of ethylene oxide.

It has now been found that the effectiveness of the bleach fix baths can be further improved, without affecting their stability, if a polyalkylene oxide is added to them in which some of the oxygen atoms are replaced by sulphur atoms. This class of substances may be characterised by the following general formula:



wherein  $\text{R}$ ,  $\text{R}'$ ,  $\text{R}''$  and  $\text{R}'''$  represent bivalent organic radicals with 2–10 carbon atoms which may be substituted,  $m$  represents an integer from 0–100,  $n$  and  $p$  an integer from 1–100,  $\text{Y}$  stands for a radical selected from the group consisting of



and mixtures thereof wherein  $\text{R}'''$  stands for a lower aliphatic radical having 1–3 carbon atoms and  $\text{X}$  represents a hydrogen atom or an aliphatic radical which may be substituted for improving the solubility of said compounds e.g. by hydroxyl, cyano, amino, carboxyl, sulfo, or a radical of an acid of phosphorus.  $\text{X}$  may further stand for an acyl radical derived from an aliphatic mono- or dicarboxylic acid.

Aliphatic, aromatic or mixed aliphatic-aromatic thioethers have proved suitable. Aliphatic thioethers which contain a plurality of thioether groupings in the molecule are preferred, however, because of their greater effectiveness. Furthermore, some of the sulphur atoms may be oxidised to sulphine or sulphonyl groups or some of the sulphur atoms may be treated with an alkylating agent to form sulphonium groups.

Examples of suitable thioethers are condensates of  $\beta,\beta'$ - and  $\gamma,\gamma'$ -dihydroxyalkyl sulphides with polyalkylene glycols, particularly the co-condensates of thiodiglycol and its alkyl-substituted products with polyethylene and/or polypropylene glycols, or the hydroxyethylation products and/or the propoxylation products of mono- and polyvalent alcohols which contain OH groups or ether oxygen atoms as solubilizing groups. Derivatives of the aforementioned polythioethers can also be used with success, for example co-condensates of the aforementioned type wherein some of the sulphur atoms have been oxidized to form sulphoxide or sulphonyl groups or in which some of the sulphur atoms have been converted by alkylation agents into sulphonium groups, or in which the OH groups have been wholly or partially esterified or etherified.

Some of these substances and a process for the production thereof are described in United States Patent Specifications Nos. 2,484,369 and 2,518,245 and in French Patent Specification 1,201,171.

Examples of such thioethers are:

(1) A condensation product containing 3.8% of sulphur, having a molecular weight of 1700 and which has been prepared from 1 mol of a polyethylene oxide having a molecular weight of 1130 and 1.27 mols of thiodiglycol.

(2) A condensation product containing 3.8% of sulphur, having a molecular weight of 1540 and which has been prepared from 1 mol of a polyethylene oxide having a molecular weight of 680 and 0.94 mol of thiodiglycol.

(3) A condensation product containing 3.7% of sulphur, having a molecular weight of 740 and which has been prepared from 1 mol of octaethylene glycol and 0.54 mol of thiodiglycol.

(4) A condensation product as recited under heading 2 in which the OH groups have been converted into the semi-ester with maleic anhydride.

(5) A condensation product as recited under heading 2 in which the OH-groups have been esterified with acetic acid.

(6) A condensation product having a molecular weight of 4000 and which has been prepared from 10 mols of thiodiglycol and 1 mol of a polyethylene oxide having a molecular weight of 1700, the terminal groups of the condensation product being esterified with maleic anhydride.

(7) A condensation product having a molecular weight of 4000 and containing 10% of sulphur, 20% of which has been converted into the methosulphate with dimethyl sulphate, said condensation product having been prepared from 10 mols of thiodiglycol and 1 mol of a polyethylene oxide having a molecular weight of 1700.

(8) A condensation product having a molecular weight of 4000 and containing 10% of sulphur, 40% of which has been converted into the sulphoxide, said condensation product having been prepared from 10 mols of thiodiglycol and 1 mol of a polyethylene oxide having a molecular weight of 1700.

(9) A thioether having terminal butyl groups, a molecular weight of approximately 2400 and containing 3% of sulphur, the thioether having been produced by the condensation of 1 mol of diethylene glycol monobutyl ether with 3 mols of thiodiglycol and 0.5 mol of a polyethylene oxide of molecular weight 1750.

(10) A polyether thioether having a molecular weight of 3000 and containing 3.3% of sulphur, said polyether having been produced by the co-polymerisation of 0.03 mol of butane-1,4-diol, 2 mols of ethylene oxide and 0.1 mol of ethylene sulphide.

(11) A polyether thioether having a molecular weight of approximately 3500 and containing 9% of sulphur, said polyether thioether having been produced by the co-polymerisation of 0.03 mol of butane-1,4-diol, 2 mols of ethylene oxide and 0.4 mol of ethylene sulphide.

(12) A condensation product having a molecular weight of 4000 and which has been produced from one mol of a polyethylene oxide of molecular weight 680 and 0.76 mol of thiodiglycol, the terminal OH groups in the condensation product having been etherified by the addition of acrylonitrile in the presence of an alkali.

(13) A thioether having terminal amino groups and 50 which has been produced by the hydrogenation of the product recited under heading 12.

(14) Dithiodiglycol HOCH<sub>2</sub>CH<sub>2</sub>S.S.CH<sub>2</sub>CH<sub>2</sub>OH

(15) A condensation product prepared from 0.94 mol of thiodiglycol and 1 mol of polyethylene oxide having a 55 molecular weight of 680, the terminal OH-groups of which being etherified with acrylonitrile and the nitrile groups saponified to form terminal  $\beta$ -carboxyethyl-groups.

(16) A condensation product being produced from 10 mols of  $\beta,\beta'$ -dimethyl-thioglycol and 1 mol of polyethylene oxide having a molecular weight of 1700, the terminal OH-groups of which are reacted with butane sultone to form terminal sulfobutyl groups.

(17) A condensation product prepared from 10 mols of thiodiglycol and 1 mol of polyethylene oxide with a molecular weight of 1700, the terminal OH-groups of which being transformed with thionylchloride into the corresponding chloride which is reacted with triethylphosphite to form terminal phosphoric acid groups.

(18) A condensation product prepared from 10 mols of thiodiglycol and 1 mol of a co-polymerise of 1 mol of propylene oxide and 9 mols of polyethylene oxide having a molecular weight of 1700.

(19) A condensation product having a molecular weight of 5200 and being prepared from 1 mol of oxethylated

resorcin having a molecular weight of 1700 and 4 mols of thiodiglycol.

In the following Tables 1 and 2, are given density values which were obtained by measuring a fixed field of photometric test wedges which were produced with an ordinary commercial colour-negative film and processed in bleach fix baths with various additives, behind a strict blue filter.

The polyethylene oxide which was used for the experiments in Table I was an addition product of 1 mol of ammonia and from 25 to 30 mols of ethylene oxide.

TABLE 1

| Processing of the film with a<br>bleach fix bath: | Density behind a<br>blue filter |
|---------------------------------------------------|---------------------------------|
| Without polyethylene oxide                        | 2.70                            |
| With 0.1 g. polyethylene oxide                    | 2.35                            |
| With 0.5 g. polyethylene oxide                    | 2.20                            |
| With 1.0 g. polyethylene oxide                    | 2.15                            |
| With 2.5 g. polyethylene oxide                    | 2.10                            |

The difference of 0.6 between the maximum and minimum values of the densities behind a blue filter represents a measure of the unbleached residual image of the field in question of a photometric test wedge processed with a bleach fix bath without an additive.

From Table 1 it can be seen that an addition of at least 1 g. of polyethylene oxide is necessary in order to permit bleaching of the residual image.

Table 2 shows the corresponding density values which were obtained in a series of experiments with polyethylene oxides with and without sulphur. The amount of polythioether being added was always 0.01 g. per liter of bleach fix bath.

It is readily apparent from Table 2 that the same bleaching effect is obtained with a considerably smaller quantity of polyethylene oxide containing sulphur than in the case of the polyethylene oxides which contain no sulphur.

TABLE 2

| Processing of the film with<br>a bleach fix bath: | Density behind a<br>blue filter |
|---------------------------------------------------|---------------------------------|
| Without additive                                  | 2.7                             |
| With 1 g. polyethylene oxide                      | 2.15                            |
| With 0.01 g. of condensation:                     |                                 |
| Product No. 1                                     | 2.08                            |
| Product No. 2                                     | 2.2                             |
| Product No. 3                                     | 2.10                            |
| Product No. 4                                     | 2.15                            |
| Product No. 5                                     | 2.30                            |
| Product No. 6                                     | 2.13                            |
| Product No. 7                                     | 2.16                            |
| Product No. 8                                     | 2.25                            |
| Product No. 9                                     | 2.15                            |
| Product No. 10                                    | 2.15                            |
| Product No. 11                                    | 2.05                            |
| Product No. 12                                    | 2.14                            |
| Product No. 13                                    | 2.15                            |

## Example 1

A photometric test wedge is exposed on an ordinary commercial two-layer negative colour film. The film is then developed at 18° C. for five minutes in a colour developer of the following composition:

2.75 g. diethyl-p-phenylenediamine sulphate  
1.2 g. hydroxylamine sulfate  
2 g. sodium sulphite (anhydrous)  
2 g. sodium hexametaphosphate  
75 g. potassium carbonate  
2 g. potassium bromide

The film is then washed for 15 minutes in running water, bleached and fixed in a bath of the following composition:

40 g. of the sodium salt of the iron (III) complex of ethylenediamine tetra-acetic acid

9 g. of the tetrasodium salt of ethylenediamine tetra-acetic acid containing about 30% active ethylenediamine tetra-acetic acid (Trilon B of the BASF)  
 3.78 g. of free ethylenediamine tetra-acetic acid  
 10 g. of sodium sulphite  
 200 g. of crystalline sodium thiosulphate  
 Water to make up to 1 litre

If 0.01 g. of a condensate of molecular weight 1700 and containing 3.8% of sulphur and which has been prepared from 1.27 mols of thiodiglycol and 1 mol of a poly-ethylene oxide of molecular weight 1130 is added to this bleach fix bath per litre, a film is obtained after 8 minutes which is free from any residual image.

If this additive is omitted, then a film which displays a considerable residual image is obtained after the bleach fix.

*Example 2*

An ordinary commercial hard grade colour paper is exposed behind a blue colour separation wedge and developed in the colour developer employed in Example 1. The sample is then treated for 5 minutes in a stop fix bath which has been prepared by dissolving 5 g. of anhydrous sodium acetate, 10 g. of sodium bisulphite and 120 g. of anhydrous sodium thiosulphate in 600 ml. of water and making up to 1 liter with water. The pH value of the bath is 6.0.

The sample is passed into the bleach fix bath employed in Example 1 without intermediate washing. If 1.0 g. of a condensate of molecular weight 1700 and containing 3.8% of sulphur and which has been prepared from 1.27 mols of thioglycol and 1 mol of a polyethylene oxide of molecular weight 1130 is added to the bleach fix bath a perfectly bleached yellow wedge is obtained after 8 minutes.

If 1.0 g. of a sulphur-free polyethylene oxide, for example an addition product of 1 mol of ammonia and from 20 to 30 mols of ethylene oxide is added instead of the polyethylene thioether containing sulphur, the yellow wedge still displays considerable remains of the silver image after a reaction time of 12 minutes.

Having thus described our invention we now state that we believe our invention to be capable of numerous variations. For example any water-soluble thiosulphates may be used as fixing agents such as alkali thiosulphates or ammonium thiosulphate. The bleach fixing bath may contain as stabilising agents any water-soluble sulfite, bisulfite or metasulfite. Furthermore the bleach fixing bath may have an additional content of water-soluble iodides as described in copending application Ser. No. 95,735, filed March 14, 1961, by Bernard Morcher, Karl Frank and Max Heilmann.

Moreover it is clear to those skilled in the art that the photographic material which shall be treated by the bleach fixing bath according to the invention may be developed by means of any developer composition known per se.

The pH-value of the bleach fixing bath according to the invention may range approximately from 5 to 8.

As to the amounts of the sulphur containing polyalkylene-oxides being added to the bleach fixing bath according to the invention it is self-evident that smaller amounts than 0.01 g./l. of the bleach fixing bath are less effective. Higher amounts may be added. The upper limit of the amount to be added is given by the solubility of said compounds, which depends on the molecular weight, the content of water-solubilizing groups and so on.

We claim:

1. In a process for the bleaching and fixing of a photographic silver halide emulsion which comprises subjecting the said emulsion to treatment with a fixing-bleaching composition comprising

(a) a conventional bleaching agent of the group consisting of complex salts of trivalent iron and an acid of the group consisting of polycarboxylic acids and nitrogen-containing polycarboxylic acids, and

(b) a conventional fixing agent consisting of a water-soluble salt of thiosulfuric acid,

the improvement of subjecting the said emulsion to treatment with a fixing-bleach composition which contains in dissolved form, in addition to the two foregoing conventional ingredients, at least 0.01 gram per liter of a substance of the group consisting of polyalkylene oxides having the formula:

10 wherein R, R', R'' and R''' are each a radical of the group consisting of alkylene radicals having up to 10 carbon atoms and phenylene, m is an integer from 0 to 100, n and p are each an integer from 1 to 100, Y is a 15 radical of the group consisting of



20 in which  $R''''$  is a lower aliphatic radical having up to 3 carbon atoms and X is a radical of the group consisting of (I) hydrogen, (II) alkyl containing up to 10 carbon atoms, (III) alkyl containing up to 10 carbon atoms and containing a substituent of the group consisting of cyano, 25 amino, carboxyl, sulfo and radicals derived from acids of phosphorous, (IV) aryl, (V) aryl radicals containing a substituent of the group consisting of amino, carboxyl, sulfo and radicals derived from acids of phosphorous, and (VI) acyl radicals of aliphatic monocarboxylic acids and aliphatic dicarboxylic acids, and mixtures thereof

**2. A bleaching and fixing composition for treating photographic silver halide emulsions comprising**

Photographic silver halide emulsions comprising  
35 (a) a conventional bleaching agent of the group consisting of complex salts of trivalent iron and an acid of the group consisting of polycarboxylic acids and nitrogen-containing polycarboxylic acids,  
(b) a conventional fixing agent consisting of a water-soluble salt of thiosulfuric acid, and  
40 (c) in dissolved form at least 0.1 gram per liter of a substance of the group consisting of polyalkylene oxides having the formula:

45 wherein R, R', R'' and R''' are each a radical of the group consisting of alkylene radicals having up to 10 carbon atoms and phenylene, m is an integer from 0 to 100, n and p are each an integer from 1 to 100, Y is a radical of the group consisting of



55 in which  $R''''$  is a lower aliphatic radical having up to 3 carbon atoms and X is a radical of the group consisting of (I) hydrogen, (II) alkyl containing up to 10 carbon atoms and (III) alkyl containing up to 10 carbon atoms and containing a substituent of the group consisting of cyano, amino, carboxyl, sulfo and radicals derived from acids of phosphorus, (IV) aryl, (V) aryl radicals containing a substituent of the group consisting of amino, carboxyl, sulfo and radicals derived from acids of phosphorus, and (VI) acyl radicals of aliphatic monocarboxylic acids and aliphatic dicarboxylic acids, and mixtures thereof.

60

65

3. A bleaching and fixing composition for the treatment of photographic silver halide emulsions comprising an aqueous solution containing the following substances in approximately the quantities specified per liter of solution:

(i) 40 grams of the sodium salt of the ferric complex of ethylenediaminetetraacetic acid,  
(ii) 9 grams of the tetrasodium salt of ethylenediaminetetraacetic acid containing approximately 30% by weight of active ethylenediaminetetraacetic acid.

- (iii) 3.78 grams of ethylenediaminetetraacetic acid,
- (iv) 10 grams of anhydrous sodium sulfite,
- (v) 200 grams of sodium thiosulfate pentahydrate, and
- (vi) 0.01 gram of condensation product having a molecular weight of 1700 and containing 3.8% by weight of sulfur that was prepared from thiodiglycol and polyethylene oxide having a molecular weight of 1300 in the proportions of 1.27 mols of thiodiglycol per mol of the polyethylene oxide.

5

## References Cited by the Examiner

## FOREIGN PATENTS

- |         |        |          |
|---------|--------|----------|
| 545,083 | 8/1957 | Canada.  |
| 866,605 | 2/1953 | Germany. |
| 966,410 | 8/1957 | Germany. |

NORMAN G. TORCHIN, *Primary Examiner.*HAROLD N. BURSTEIN, *Examiner.*